

1

2,743,172

PROCESS OF PREPARING INDURATED PELLETS  
OF IRON ORE FINES

Fred D. De Vaney, Hibbing, Minn., assignor to Erie Mining Company, Hibbing, Minn., a corporation of Minnesota

No Drawing. Application January 28, 1952,  
Serial No. 268,681

1 Claim. (Cl. 75—3)

This invention relates to an improvement in the art of agglomerating finely divided iron ore material, especially finely divided iron ore concentrates, by the so-called "pelletizing" process involving forming the finely divided material in moist state into small balls or pellets by a rolling operation and thereafter heat-treating (indurating) the pellets in a shaft-type furnace to impart to them a considerable mechanical strength or ruggedness. An article by C. V. Firth published in the April 20, 1944, issue of "Proceedings of the Blast Furnace and Raw Materials Committee," A. I. M. M. E., provides a general description of the pelletizing process. The present invention is more particularly concerned with improvements in that type of pelletizing process wherein the small balls or pellets contain uniformly dispersed therethrough a normally solid exothermically oxidizable component in an amount insufficient per se to yield by its oxidation all of the heat required for carrying out the induration step. The invention comprises process and product aspects.

Because of the peculiar heating cycle inherent in indurating such pellets in a shaft furnace, the pellets have a great tendency to disintegrate during the earlier stages of the induration procedure which tendency is not encountered in more gradual heating as in a tunnel kiln or the like. Thus, they may exfoliate or they may explosively rupture during the rapid heating. Moreover, such pellets are readily susceptible, while in moist state, to deformation and to formation of aggregations of pellets, as when, prior to incipient induration, the moist pellets are subjected to the pressure of a considerable mass of superimposed pellets.

It has now been found that the above disadvantages can be avoided by homogeneously incorporating with the moist finely divided ore particles, prior to balling up, a very small amount of bentonite. The amount of bentonite so used must be controlled within narrow limits, viz., within the limits 0.1% and 1.0% by weight based on the dry weight of the ore particles. Less than 0.1% bentonite does not produce a useful result. If more than 1.0% bentonite is used the resulting moist mixture when subjected to balling-up in the balling drum quickly balls up but the resulting product consists of undesirably small balls which cannot be made to "grow," by accretion, to a size useful in feeding the blast furnace. The optimum amount of bentonite addition is about 0.5% by weight, i. e., about 10.0 pounds per long ton, dry weight, of the ore fines to be pelletized.

Ore concentrates pellets containing 0.1%—1.0% of bentonite are not sticky as freshly formed, and the freshly formed pellets do not acquire stickiness during such handling as is required for transferring the pellets to the top of the induration furnace and for laying down a layer of the moist pellets on the stockline of the column of pellets undergoing heat-treatment in the furnace. This small content of bentonite very materially adds to the mechanical strength or ruggedness of the "raw" (i. e., freshly formed and unheated) pellets, which added mechanical strength carries through the drying of the pellets

2

and into the incipient induration stage of the heat treatment. Very surprisingly, this small content of bentonite materially increases the "fired strength" of the pellets, that is to say, the ultimate mechanical strength and ruggedness of the discharged fully indurated and cooled pellets. This fired strength is not diminished by weathering of the pellets. This increase in fired strength usually amounts to between 10% and 20%.

Bentonite, as used in the present relation, is much superior to other types of clay—the superiority being due in part to the gel-forming properties of bentonite and in part to the fine particle size of the bentonite, which latter has about 7 times the surface area of the next-nearest clay.

Average number of grains per linear centimeter:

|            |        |
|------------|--------|
| Bentonite  | 20,000 |
| Ball clay  | 3,400  |
| Brick clay | 2,600  |
| China clay | 2,400  |

Bentonite exhibits greater mobility in the moist state and tends to film out over a tremendous surface area. This film, in the case of bentonite-containing iron ore pellets, reacts, at induration temperature, with  $Fe_3O_4$  or  $Fe_2O_3$  or/and with gangue components to produce a thin coating of slag covering the iron oxide grains and firmly bonding the mass together. Moreover, many iron ore concentrates are deficient in alumina, so that the small addition of bentonite contributes a little needed alumina to the fired product.

It has been found that use of bentonite is attended by two desirable results, viz., (a) the same contributes to the temporary strength of the pellets, i. e., to the pellets as freshly formed and during handling of the latter and through the drying out of the pellets in the beginning of the induration operation which drying period marks the level of greatest fragility of the pellets, and (b) the same contributes a remarkable increase in the final, or "fired," strength of the pellets. This increase in fired strength usually amounts to an improvement of between 10% and 20%. In a case where the dry strength of the pellets is of the order of 1 lb. per pellet in the absence of bentonite, use of bentonite within the amount range specified increases the dry strength to 20 lbs. or more—sometimes to as much as 50 lbs. per pellet.

The improvement in fired strength through use of bentonite is in sharp contrast with the effect of other earthy materials such as barite and clays other than bentonite. Ordinary clays do not improve either the fired strength or the dry strength of an iron ore pellet, while use of barite depreciates rather than improves the strength of the pellets.

Use of bentonite in iron ore pellets normally increases the drop test value from an average of 85% to an average of 91.5%. This decrease in fines production during induration improves the furnacing operation by decreasing the furnace pressures materially.

The invention will now be described in greater particularity with reference to the following illustrative examples:

## Example I

A. The starting material was a filter cake of magnetic concentrates obtained from a magnetic taconite found in the Mesabi range. The material analyzed as follows:

|           | Per cent |
|-----------|----------|
| Fe        | 66.13    |
| P         | 0.017    |
| $SiO_2$   | 4.86     |
| Mn        | 0.18     |
| $Al_2O_3$ | 0.12     |

the iron being present mostly in the form of magnetite,  $Fe_3O_4$ , and the particle size distribution was as follows: essentially all minus 100 mesh and 68% finer than 325 mesh.

The filter cake was divided into a number of portions one of which was processed as a check. To another portion there was added bentonite in an amount to give a 0.5% concentration of the bentonite on the dry basis, and the bentonite-containing material was mixed until the bentonite was found to be homogeneously dispersed throughout the mass.

Thereupon, the pugged material was fed to a balling drum wherein the material was formed into pellets. The finished pellets varied somewhat in size within the limits 1.5 inches and 0.5 inch, averaging about 1.125 inches in diameter. They were found to have, in the natural wet state, a compressive strength of 6.2 pounds per pellet, and in the dry state (dried to 230° F.) a compressive strength of 21.5 pounds per pellet.

The resulting pellets were transferred to the top of a shaft-type indurating furnace generally similar to that disclosed in U. S. Patent No. 2,533,142 to Percy H. Royster and, at substantially room temperature (60° F.) were laid down on the stockline of a column of similar pellets undergoing heat-treatment. The furnace had a cross-sectional area of about 4.95 square feet at the mouth, and was fed at a rate to yield 2150 pounds per hour of indurated and cooled, dry pellets. The gases moving from the combustion chamber to and into the column at the level of the bottom of the upper of the two chambers of the furnace were maintained at a temperature of about 1850° F. by suitable adjustment of the rate of feed of the fuel. The average fuel oil feed was 2.5 gallons/hour. The rate of blowing of the air was about 452 C. F. M. (cubic feet per minute). The top temperature attained by the pellets in the upper chamber of the furnace was about 2340° F., which top temperature was attained about 12 inches below the stockline. At the level at the bottom of the upper chamber the pellets had a temperature of about 1925° F. The exit gas temperature was estimated as 245° F.

The product discharged from the induration furnace at a temperature of about 275° F., and was found to have the following screen analysis:

|                | Per cent |
|----------------|----------|
| Plus 1 inch    | 53.5     |
| Plus .75 inch  | 26.3     |
| Plus .5 inch   | 12.2     |
| Plus 10 mesh   | 4.5      |
| Plus 100 mesh  | 2.3      |
| Minus 100 mesh | 1.2      |

This product was subjected to a "drop test" in which 100 pounds of pellets, all 0.5 inch diameter and larger, were dropped five (5) times through a pipe 32 feet tall onto a steel plate, and then screened at 10 mesh and the amount of minus 10 mesh material determined by weighing. Pellets to be suitable for lake shipment must not show more than 12% by weight of minus 10 mesh material when tested by this method. The above-described fired product tested 91.5%, i. e., it contained only 8.5% of minus 10 mesh material.

B. The above mentioned "check" portion was similarly balled up in the balling drum, fed to and indurated in the induration furnace and thereafter examined. The moist raw pellets ranged in size as above, and averaged as above in diameter, and had a compressive strength of 2.15 lbs. per pellet in the wet state and of 1.05 lbs. per pellet in the dried state. The pellets were subjected to the same induration treatment as that described above. The product discharged from the furnace had the following screen analysis:

|                | Per cent |
|----------------|----------|
| Plus 1 inch    | 40.9     |
| Plus .75 inch  | 27.5     |
| Plus .5 inch   | 12.5     |
| Plus 10 mesh   | 8.5      |
| Plus 100 mesh  | 6.2      |
| Minus 100 mesh | 4.4      |

and showed a drop test of about 85.4%, i. e., 14.6% of minus 10 mesh material.

It will be appreciated that use of the small amount of bentonite (Experiment A) made the wet pellets measurably stronger, and conferred a remarkably higher dry strength, that the disintegration losses during induration were smaller, and that the final product was very materially stronger. Because of lack of degradation the furnace pressures were reduced about 60%.

In another, companion, test 22.5 lbs. bentonite were added. The resulting balls were small, not averaging more than 0.5 inch in size. Because of this size limitation the material was not further processed.

#### Example II

The starting material was a magnetic concentrate from Mahoning taconite (St. Louis County, Minnesota, U. S. A.), the same having substantially the same composition and screen analysis as that of the starting material referred to in Example I. The magnetic concentrate was thoroughly mixed with 15% water by weight and with 0.5% by weight of bentonite, and the uniform mixture was rolled into balls. The balled-up material was heated in a muffle furnace for 5.5 hours at 1000° C. The fired product showed no cracks or disintegration, and withstood dropping from a height of 10 feet without breakage.

In a repetition of this experiment 1.0% bentonite was used with equally good results.

#### Example III

The starting material was a finely divided flotation concentrate made from a tailing, containing 58.1% iron: the iron minerals were hematite and limonite with hematite predominating. The grain size was approximately all minus 100 mesh, but only 51% was finer than 325 mesh and with only a minor amount of colloidal fines.

This starting material was thoroughly mixed with approximately 11% of water and 11 pounds per long ton of anthracite fines, and divided into portions.

One portion was subjected to the balling-up operation described in Example I above. Because of the granular nature of the solids, the balls were very fragile and the amount of degradation was excessive: consequently, the test was discontinued.

Into another portion of the above mixture there was homogeneously dispersed 10 pounds per long ton of bentonite, and the resulting mixture was formed into pellets in the manner described in Example I above. The pellets averaged  $\frac{1}{8}$  inch in diameter. A test showed that in their dry state the pellets had a compressive strength of 3.5 lbs./pellet.

The pellets were transferred to the induration furnace wherein they were subjected to induration treatment after the manner described in Example I above. Fuel oil in the average amount of 2.8 gallons/hour was fed to the combustion chamber to maintain the temperature of 1950° F. in the air-gaseous combustion products mixture exiting from the combustion chamber and into the bottom of the upper chamber of the furnace.

There was little degradation in the furnace, and the fired product contained less than 5% of minus 10 mesh material. The drop test on this material showed about 92% on 10 mesh.

The use of an exothermically oxidizable component in the bentonite-containing pellets makes possible the occurrence, in the upper part of that portion of the column occupying the upper chamber of the furnace, a top tem-

perature materially higher than that of the air-gaseous combustion products mixture introduced (from the combustion chamber) at the bottom of the upper chamber. This "flash" top temperature preferably is caused to be sufficiently high that sintering or partial fusion occurs in the interiors of the pellets, while the exteriors of the pellets are swept by gases which while being hot have a cooling effect on said exteriors preventing the latter from becoming molten or sticky. Examination of pellets so indurated shows that the particles resident in the exterior "shells" of the pellets are not materially sintered together whereas the particles occupying the interiors of the pellets have experienced partial fusion. Fused slag is readily discernible in the pellets' interiors, said slag being in the interstices between, and bonding together, the iron oxide particles. This slag bond between iron oxide particles is very strong. The bentonite tends to produce a slag having a melting point materially lower than if the normal ore components only are present. Hence, the slag bond develops at a temperature below dangerous melting temperature of the iron oxide.

I claim:

Process of preparing indurated pellets of finely divided iron ore concentrates which comprises forming a homogeneous plastic mixture consisting essentially of the finely divided iron ore concentrates, approximately 11% of water and from about 0.5% to not materially in excess of 1.0% by weight of bentonite based on the dry weight of

the finely divided iron ore concentrates, forming the resulting homogeneous mixture into small masses, protractedly rolling the small masses in an inclined rotary drum into raw pellets averaging between 1.5 inches and 0.5 inch in a diameter, and subjecting an assemblage of the raw pellets to thermal hardening treatment during which the raw pellets are dried and thereupon are heated, in contract with an oxidizing gaseous heat exchange medium at an elevated temperature, to an induration temperature of at least 1000° C. but below the normal fusing point of the iron ore, at which induration temperature a bentonite slag bond is formed within the interiors of the pellets, thereby producing an indurated product consisting essentially of discrete indurated pellets of iron ore.

15

References Cited in the file of this patent

UNITED STATES PATENTS

|           |                |       |               |
|-----------|----------------|-------|---------------|
| 2,279,033 | Dolbear        | ----- | Apr. 7, 1942  |
| 2,357,198 | Hooey          | ----- | Aug. 29, 1944 |
| 2,533,142 | Royster        | ----- | Dec. 5, 1950  |
| 2,582,386 | Komarek et al. | ----- | Jan. 15, 1952 |

OTHER REFERENCES

25 U. S. Bureau of Mines Report of Investigation 4829, published December 1951, by Bureau of Mines, Washington, D. C., page 1, Figures 4 and 8 and pages 7 and 8 pertinent. Entire report 17 pages and 5 sheets of drawing.